# EUROPEAN PATENT APPLICATION

(11) **EP 4 786 628 A1**
(43) Date of publication of application: **05.08.2026**
(21) Application number: 24872576.4
(22) Date of filing: 27.09.2024
(51) Int. Cl.: C22C 38/00, C21D 8/12, C21D 9/46, C22C 38/60, H01F 1/147, H01F 27/245, H01F 41/02

(54) **GRAIN-ORIENTED ELECTROMAGNETIC STEEL SHEET AND METHOD FOR MANUFACTURING GRAIN-ORIENTED ELECTROMAGNETIC STEEL SHEET**

(30) Priority: 27.09.2023 JP 2023166173
(71) Applicant: Nippon Steel Corporation, Tokyo 100-8071 (JP)
(72) Inventor: MATSUBARA, Ryo, Tokyo 100-8071 (JP); KAWAMURA, Yusuke, Tokyo 100-8071 (JP); HONMA, Rei, Tokyo 100-8071 (JP); SUZUMA, Toshiyuki, Tokyo 100-8071 (JP)
(74) Representative: Vossius & Partner Patentanwälte Rechtsanwälte mbB
(86) International application number: PCT/JP2024/034822
(87) International publication number: WO 2025/070796

(57) **Abstract**

This grain-oriented electrical steel sheet is a grain-oriented electrical steel sheet having a magnetic domain control treatment line on a surface thereof, |α_{All}|-lα_{Dr}| ≥ 0.1° is satisfied, |α_{All}| is an average value of absolute values of α angles over an entire surface of the grain-oriented electrical steel sheet, and |α_{Dr}| is an average value of absolute values of α angles at magnetic domain control points that are intersection points of a plurality of the imaginary lines set at intervals of 2 mm in parallel along a rolling direction of the grain-oriented electrical steel sheet and the magnetic domain control treatment line. A method for manufacturing a grain-oriented electrical steel sheet according to another aspect of the present disclosure includes: a step of measuring a distribution of α angles on a surface of an original sheet of a grain-oriented electrical steel sheet; a step of specifying a region where an absolute value of the α angle is 5° or less; and a step of applying a magnetic domain control treatment to the region where the absolute value of the α angle is 5° or less.

## Description

### TECHNICAL FIELD

The present invention relates to a grain-oriented electrical steel sheet and a method for manufacturing a grain-oriented electrical steel sheet.

Priority is claimed on Japanese Patent Application No. 2023-166173, filed in Japan on September 27, 2023, the content of which is incorporated herein by reference.

### BACKGROUND ART

The grain-oriented electrical steel sheet is a steel sheet containing 7 mass% or less of Si and having a secondary recrystallization structure in which secondary recrystallized grains are accumulated in a {1101<001> orientation (Goss orientation) in which an easy axis of magnetization <001> is oriented in a rolling direction. Grain-oriented electrical steel sheets are mainly used as iron cores of power transformers. Grain-oriented electrical steel sheets are required to reduce energy loss (iron loss).

A technique of narrowing a spacing of magnetic domain walls of a grain-oriented electrical steel sheet (magnetic domain refinement technique by magnetic domain control treatment) for reducing iron loss has been known for a long time. The spacing of magnetic domain walls can be narrowed by irradiating the surface of the grain-oriented electrical steel sheet with a laser or an electron beam in a direction intersecting the rolling direction to introduce a thermal strain. The spacing of magnetic domain walls can also be narrowed by forming a groove in the direction intersecting the rolling direction on the surface of the grain-oriented electrical steel sheet. Examples of a method of forming the groove include a method of irradiating a laser or an electron beam, a method by mechanical processing such as gear, and a method by chemical processing such as etching.

In recent years, in order to provide a grain-oriented electrical steel sheet having good iron loss characteristics, various improved techniques related to magnetic domain refinement have been proposed (see, for example, Patent Documents 1 to 3.).

### Citation List

### Patent Documents

Patent Document 1: Japanese Unexamined Patent Application, First Publication No. 2012-57219
Patent Document 2: Japanese Unexamined Patent Application, First Publication No. 2012-12664
Patent Document 3: Japanese Unexamined Patent Application, First Publication No. 2012-57218

### SUMMARY OF INVENTION

### Technical Problem

When the magnetic domain control treatment is applied to the grain-oriented electrical steel sheet, the magnetostrictive characteristic of the grain-oriented electrical steel sheet changes depending on the flux closure domain. As a result, noise characteristics of the grain-oriented electrical steel sheet deteriorate. The noise characteristic is a degree of noise generated by an electrical product (for example, a transformer, a motor, and the like) manufactured using a grain-oriented electrical steel sheet as a material. Magnetostriction is a phenomenon in which an outer shape is slightly deformed when a ferromagnetic material is magnetized. When the grain-oriented electrical steel sheet is excited by alternating current, the magnitude of the magnetostriction changes with a change in the strength of magnetization, and thus vibration occurs. The magnitude of the magnetostriction is very small on the order of 10-6, but the magnetostriction generates vibration in the iron core, and the vibration propagates to an external structure such as a tank of a transformer to become noise.

That is, the magnetic domain control treatment is effective for suppressing iron loss of the grain-oriented electrical steel sheet, but deteriorates noise characteristics of the grain-oriented electrical steel sheet. In recent years, there is an increasing demand for not only a reduction in iron loss but also a reduction in noise for grain-oriented electrical steel sheets. However, no magnetic domain refinement technique capable of achieving both noise reduction and iron loss reduction has been proposed so far.

An object of the present disclosure is to provide a grain-oriented electrical steel sheet capable of achieving both iron loss reduction and noise reduction, and a manufacturing method therefore.

### Solution to Problem

The gist of the present disclosure is as follows.
(1) A grain-oriented electrical steel sheet according to an aspect of the present disclosure is a grain-oriented electrical steel sheet having a magnetic domain control treatment line on a surface thereof, wherein |α_{All}|-lα_{Dr}| ≥ 0.1° is satisfied, |α_{All}| is an average value of absolute values of α angles over an entire surface of the grain-oriented electrical steel sheet, and |α_{Dr}| is an average value of absolute values of α angles at magnetic domain control points that are intersection points of a plurality of imaginary lines set at intervals of 2 mm in parallel along a rolling direction of the grain-oriented electrical steel sheet and the magnetic domain control treatment line.
(2) Preferably, the grain-oriented electrical steel sheet according to (1) satisfies |α_{All}|-|α_{Dr}| ≥ 0.2°.
(3) Preferably, the grain-oriented electrical steel sheet according to (1) satisfies |α_{All}|-|α_{Dr}| ≥ 0.5°.
(4) Preferably, the grain-oriented electrical steel sheet according to (1) satisfies |α_{All}|-|α_{Dr}| ≥ 1.0°.
(5) Preferably, the grain-oriented electrical steel sheet according to any one of (1) to (4) satisfies |γ_{All}|-|α_{Dr}| ≥ 0.1°, and |γ_{All}| is an average value of absolute values of γ angles over the entire surface of the grain-oriented electrical steel sheet.
(6) Preferably, the grain-oriented electrical steel sheet according to any one of (1) to (5) satisfies σα_{Dr} < σα_{All}, σα_{All} is a standard deviation of the absolute value of the α angle over the entire surface of the grain-oriented electrical steel sheet, and σα_{Dr} is the standard deviation of the absolute value of the α angle at the magnetic domain control point.
(7) Preferably, in the grain-oriented electrical steel sheet according to any one of (1) to (6), the magnetic domain control treatment line is a groove.
(8) A method for manufacturing a grain-oriented electrical steel sheet according to another aspect of the present disclosure includes: a step of measuring a distribution of α angles on a surface of an original sheet of a grain-oriented electrical steel sheet; a step of specifying a region where an absolute value of the α angle is 5° or less; and a step of forming a magnetic domain control treatment line in the region where the absolute value of the α angle is 5° or less.
(9) Preferably, in the method for manufacturing a grain-oriented electrical steel sheet according to (8), the magnetic domain control treatment is applied by irradiation with a laser or an electron beam.

### Advantageous Effects of Invention

According to the present disclosure, it is possible to provide a grain-oriented electrical steel sheet capable of achieving both iron loss reduction and noise reduction, and a method for manufacturing the same.

### BRIEF DESCRIPTION OF DRAWINGS

[FIG. 1] A plan view of a grain-oriented electrical steel sheet according to an embodiment of the present disclosure.
[FIG. 2] A plan view of a normal grain-oriented electrical steel sheet.
[FIG. 3] A schematic diagram illustrating an example of a constitution of a laser irradiation device.
[FIG. 4] A plan view of an original sheet of a grain-oriented electrical steel sheet.
[FIG. 5] An explanatory diagram of an imaginary line VL1 and an imaginary line VL2 set at the time of calculating |α_{All}|.

### DESCRIPTION OF EMBODIMENTS

### (1. Grain-oriented electrical steel sheet 1)

The grain-oriented electrical steel sheet 1 according to the present embodiment has a magnetic domain control treatment line 11 on the surface thereof, and satisfies |α_{All}|-|α_{Dr}| ≥ 0.1°. |α_{All}| is an average value of absolute values of α angles over the entire surface of the grain-oriented electrical steel sheet 1. |α_{Dr}| is an average value of absolute values of α angles at the magnetic domain control point VP2, which is an intersection point of a plurality of imaginary lines VL3 set at intervals of 2 mm in parallel along the rolling direction RD of the grain-oriented electrical steel sheet 1 and the magnetic domain control treatment line 11.

### (Magnetic domain control treatment line 11)

A plurality of the magnetic domain control treatment lines 11 provided on the surface of the grain-oriented electrical steel sheet 1 have a function of refining a 180° magnetic domain. By refining the magnetic domain, the iron loss of the grain-oriented electrical steel sheet 1 can be reduced. The magnetic domain is a collection of magnetic dipoles existing inside a ferromagnetic material, and is a small region where magnetic moments are aligned in one direction. The 180° magnetic domain is a magnetic domain in which the magnetization direction is the <100> orientation of the crystal and which is sandwiched between two 180° magnetic walls substantially parallel to the rolling direction RD. A distance (domain wall interval) between adjacent domain walls of the 180° magnetic domain is referred to as a spacing of the 180° magnetic domain walls.

Suitable examples of the magnetic domain control treatment line 11 are a thermal strain and a groove. By refining the magnetic domain, the iron loss of the grain-oriented electrical steel sheet 1 can be suppressed. However, the magnetic domain control treatment line 11 changes the magnetostrictive characteristic of the grain-oriented electrical steel sheet 1 according to the flux closure domain. As a result, noise characteristics of the grain-oriented electrical steel sheet 1 deteriorate.

The magnetic domain control treatment line 11 is formed in a direction intersecting the rolling direction RD of the grain-oriented electrical steel sheet 1. In the general grain-oriented electrical steel sheet 1 as exemplified in FIG. 2, the magnetic domain control treatment line 11 is formed over the entire width of the grain-oriented electrical steel sheet 1. However, in the grain-oriented electrical steel sheet 1 according to the present embodiment as exemplified in FIG. 1, it is not essential to provide the magnetic domain control treatment line 11 over the entire width of the grain-oriented electrical steel sheet 1. At least some of the magnetic domain control treatment lines 11 are interrupted in a region 12B where the α angle is large to be described later.

In the grain-oriented electrical steel sheet 1 illustrated in FIG. 1, the magnetic domain control treatment line 11 is a straight line. On the other hand, the magnetic domain control treatment line 11 may be a curve. The magnetic domain control treatment line 11 may have a shape having a straight line portion and a bent portion. The magnetic domain control treatment line 11 may be provided on one surface or both surfaces of the grain-oriented electrical steel sheet 1. When the magnetic domain control treatment line 11 is provided on both surfaces of the grain-oriented electrical steel sheet 1, various aspects of the grain-oriented electrical steel sheet 1 according to the present embodiment may be applied to at least one surface of the grain-oriented electrical steel sheet 1.

### (α angle)

In the grain-oriented electrical steel sheet 1 according to the present embodiment, the values |α_{All}| and |α_{Dr}| calculated by measuring the α angles satisfy a predetermined relational expression. The α angle is a deviation angle of crystal grains from the Goss orientation about the axis in the rolling surface normal direction ND. It is known that controlling the α angle is effective for controlling the magnetic characteristics of the grain-oriented electrical steel sheet 1. The deviation angle of the crystal grains from the Goss orientation about the axis in the transverse direction TD is referred to as a β angle, and the deviation angle of the crystal grains from the Goss orientation about the axis in the rolling direction RD is referred to as a γ angle.

The present inventors compared iron loss values of a plurality of grain-oriented electrical steel sheets 1 having different α angles before and after magnetic domain control treatment. As a result, it was found that when the magnetic domain control treatment is performed on the grain-oriented electrical steel sheet having a small α angle, the iron loss reduction effect by the magnetic domain control treatment is larger than that when the magnetic domain control treatment is performed on the grain-oriented electrical steel sheet having a large α angle. Before and after the magnetic domain control treatment, the iron loss changes, but the α angle does not change. Although the mechanism in which the iron loss reduction effect by the magnetic domain control treatment is large in the region where the α angle is small is not clear, it is considered that the deviation of the magnetization easy axis from the rolling direction is small in the region where the α angle is small, the hysteresis loss is small, and the like advantageously worked on the iron loss reduction by the magnetic domain control treatment.

On the other hand, it is considered that the magnetic domain control treatment to the region where the α angle is large and the effect of reducing the iron loss is small causes deterioration of noise characteristics due to the flux closure domain.

According to the above findings, it has been considered that both a reduction in iron loss and a reduction in noise can be achieved by preferentially performing magnetic domain control treatment on a region where the α angle is small, that is, a large iron loss reduction effect by the magnetic domain control treatment.
$\left(\left|{α}_{All}\right|-\left|{α}_{Dr}\right|\right)$

The grain-oriented electrical steel sheet 1 according to the present embodiment satisfies |α_{All}|-lα_{Dr}| ≥ 0.1°. |α_{All}| is an average value of absolute values of α angles over the entire surface of the grain-oriented electrical steel sheet 1. |α_{Dr}| is an index of an α angle in the magnetic domain control treatment line 11. Specifically,|α_{Dr}| is an average value of absolute values of α angles at the magnetic domain control point VP2, which is an intersection point of a plurality of imaginary lines VL3 set at intervals of 2 mm in parallel along the rolling direction RD of the grain-oriented electrical steel sheet 1 and the magnetic domain control treatment line 11. |α_{Dr}| is obtained by averaging the absolute values of the α angles measured at each of a plurality of the magnetic domain control points VP2. Details of the method of measuring |α_{All}| and |α_{Dr}| will be described later.

When the grain-oriented electrical steel sheet 1 satisfies |α_{All}|-|α_{Dr}| ≥ 0.1°, the magnetic domain control treatment line 11 is preferentially provided in the region 12A where the α angle is small. Generally, the grain-oriented electrical steel sheet 1 has a region 12A where the α angle is small and a region 12B where the α angle is large. In the grain-oriented electrical steel sheet 1 schematically illustrated in FIG. 1, the magnetic domain control treatment line 11 is preferentially arranged in a region 12A where the α angle is small. Therefore, |α_{Dr}|, which is an index of the α angle in the magnetic domain control treatment line 11, is smaller than the average value |α_{All}| of the α angles over the entire surface of the grain-oriented electrical steel sheet 1. On the other hand, in the normal grain-oriented electrical steel sheet 1 shown in FIG. 2, the magnetic domain control treatment lines 11 are arranged without considering the distribution of the α angles. Therefore, |α_{Dr}|, which is an index of the α angle in the magnetic domain control treatment line 11, is substantially the same value as the average value |α_{All}| of the α angles over the entire surface of the grain-oriented electrical steel sheet 1.

### (Basic principle and operation and effects)

The present inventors have found that, according to the grain-oriented electrical steel sheet 1 satisfying |α_{All}|-|α_{Dr}| ≥ 0.1°, both iron loss and noise can be reduced. This is because, in the grain-oriented electrical steel sheet 1 satisfying |α_{All}|-|α_{Dr}| ≥ 0.1°, while the magnetic domain control treatment line 11 is provided in the region 12A where the α angle is small, that is, the region having a large magnetic domain control effect, the magnetic domain control treatment for the region 12B where the α angle is large, that is, the region having a small magnetic domain control effect is suppressed.

The most basic aspect of the grain-oriented electrical steel sheet 1 according to the present embodiment has been described above. Hereinafter, a more preferred aspect will be described.

### (Preferred numerical value range of |α_{All}|-|α_{Dr}|)

The larger |α_{All}|-|α_{Dr}| is, the more preferable it is from the viewpoint of improving noise characteristics. |α_{All}|-lα_{Dr}| is more preferably, for example, 0.2° or more, 0.5° or more, or 1.0° or more. That is, it is more preferable that |α_{All}|-|α_{Dr}| ≥ 0.2°, |α_{All}|-|α_{Dr}| ≥ 0.5°, or |α_{All}|-|α_{Dr}| ≥ 1.0° is satisfied. This achieves further improvement in noise characteristics.

The upper limit of |α_{All}|-|α_{Dr}| is not particularly limited, and for example, |α_{All}|-|α_{Dr}| may be 5.0° or less, 4.0° or less, or 3.0° or less.

### (Preferred numerical value range of |γ_{All}|-|α_{Dr}|)

The grain-oriented electrical steel sheet 1 according to the present embodiment preferably satisfies |γ_{All}|-|α_{Dr}| ≥ 0.1°. |γ_{All}| is an average value of absolute values of γ angles over the entire surface of the grain-oriented electrical steel sheet 1. Details of a method of measuring |γ_{All}| will be described later. By satisfying |γ_{All}|-|α_{Dr}| ≥ 0.1°, further improvement in noise characteristics is achieved.

### (Relationship between σα_{Dr} and σα_{All})

The grain-oriented electrical steel sheet 1 preferably satisfies σα_{Dr} < σα_{All}. σα_{All} is the standard deviation of the absolute value of the α angle over the entire surface of the grain-oriented electrical steel sheet 1, and σα_{Dr} is the standard deviation of the absolute value of the α angle at the magnetic domain control points VP2, which are the intersection points of a plurality of the imaginary lines VL3 set at 2 mm intervals in parallel along the rolling direction RD of the grain-oriented electrical steel sheet 1 and the magnetic domain control treatment line 11. In the grain-oriented electrical steel sheet 1 satisfying σα_{Dr} < σα_{All}, the variation in α angle at the magnetic domain control point VP2 is smaller than the overall variation in α angle of the grain-oriented electrical steel sheet 1. That is, in this case, since the magnetic domain control treatment is intensively performed in the region where the iron loss reduction effect is large, the noise characteristics are further improved.

### (Aspect of magnetic domain control treatment line 11)

The type of the magnetic domain control treatment line 11 is not particularly limited, but suitable examples thereof are a thermal strain and/or a groove. The thermal strain can be formed using means such as laser irradiation, electron beam irradiation, and ion implantation. The groove can be formed using means such as laser irradiation, electron beam irradiation, and machining.

The thermal strain disappears by the stress relief annealing or the heat treatment according thereto. Therefore, when the grain-oriented electrical steel sheet 1 is subjected to a heat treatment, the magnetic domain control treatment line 11 is preferably a groove. On the other hand, since the thermal strain can be easily formed, when simplification of a manufacturing step is required, it is preferable to set the magnetic domain control treatment line 11 to the thermal strain. The grain-oriented electrical steel sheet 1 may include both the thermal strain and groove.

### (2. Manufacturing apparatus of grain-oriented electrical steel sheet 1)

Next, an example of a manufacturing apparatus of the grain-oriented electrical steel sheet 1 according to the present embodiment will be described. However, the manufacturing apparatus described below is merely an exemplary example. The grain-oriented electrical steel sheet 1 according to the present embodiment can be manufactured using an arbitrary device.

As means for introducing the thermal strain into the surface of the original sheet 2, known means such as laser irradiation, electron beam irradiation, and ion implantation can be adopted. As means for forming a groove on the surface of the original sheet 2, known means such as laser irradiation, electron beam irradiation, and machining can be adopted. Hereinafter, a constitution of the laser irradiation device 500 that introduces the thermal strain by laser irradiation will be described.

FIG. 3 illustrates a constitution of the laser irradiation device 500. The laser irradiation device 500 includes a polygon mirror 501, a light source device 503, a collimator 505, a condensing lens 507, a motor 509, a sensor 511, a control unit 513, and a sheet passing device 515.

The sheet passing device 515 passes the original sheet 2 in the rolling direction RD.

The polygon mirror 501 has, for example, a regular polygonal prism shape. A plurality of the plane mirrors is provided on each of a plurality of side surfaces constituting the polygon mirror 501 having a regular polygonal prism shape. The laser beam LB enters the plane mirror of the polygon mirror 501 in one direction (horizontal direction) from the light source device 503 via the collimator 505 and is reflected by the plane mirror.

The polygon mirror 501 is rotatable about the rotary shaft O1 by driving from the motor 509. The incident angle of the laser beam LB with respect to the plane mirror sequentially changes according to the rotation angle of the polygon mirror 501. As a result, the reflection direction of the laser beam LB is sequentially changed, and the surface of the original sheet 2 can be scanned. A Reference Number P in FIG. 3 represents an interval between the adjacent magnetic domain control treatment lines 11, that is, an irradiation pitch of the laser beam LB.

The light source device 503 outputs the laser beam LB by a predetermined irradiation system (for example, a continuous irradiation system or a pulse irradiation system) under the control of the control unit 513.

The condenser lens 507 is provided on the optical path of the laser beam LB reflected from the polygon mirror 501. The condenser lens 507 constitutes a condenser optical system having a predetermined focal distance. The laser beam LB reflected from the polygon mirror 501 is condensed on the surface of the original sheet 2 via the condenser lens 507, whereby the thermal strain is introduced into the surface of the original sheet 2.

The motor 509 is coupled to the polygon mirror 501. The motor 509 rotationally drives the polygon mirror 501 under the control of the control unit 513.

The sensor 511 is connected to a drive shaft of the motor 509. The sensor 511 detects a rotation angle of the polygon mirror 501 rotated by the motor 509. Furthermore, the sensor 511 outputs a signal (Hereinafter, the rotation angle signal is referred to as a rotation angle signal.) indicating the detected rotation angle to the control unit 513.

The control unit 513 includes a processor. The control unit 513 is connected to the light source device 503, the motor 509, the sensor 511, and the sheet passing device 515. The control unit 513 receives an input of a speed signal from the sheet passing device 515. Further, the control unit 513 outputs a signal instructing the motor 509 to rotationally drive the polygon mirror 501.

In addition, the control unit 513 controls on and off of the power of the laser beam LB output from the light source device 503 based on the stress introduction signal representing the magnetic domain control treatment region 21 and the rotation angle signal output from the sensor 511. The stress introduction signal is input to the laser irradiation device 500 based on position data obtained in a step of specifying a region where the absolute value of the α angle is 5° or less, which will be described later.

### (3. Method for manufacturing grain-oriented electrical steel sheet 1)

Next, a method for manufacturing the grain-oriented electrical steel sheet 1 according to the present embodiment will be described. According to the method for manufacturing a grain-oriented electrical steel sheet 1 according to the present embodiment, the grain-oriented electrical steel sheet 1 according to the present embodiment can be suitably manufactured. However, the manufacturing method described below is merely an example of a suitable manufacturing method of the grain-oriented electrical steel sheet 1, and does not limit the grain-oriented electrical steel sheet 1. For convenience of description, the manufacturing apparatus will be appropriately referred to in the description of the manufacturing method. However, the manufacturing apparatus mentioned below is merely a preferred example for carrying out the method for manufacturing the grain-oriented electrical steel sheet 1 according to the present embodiment.

A method for manufacturing a grain-oriented electrical steel sheet 1 according to the present embodiment includes: a step of measuring an α angle; specifying a region where an absolute value of the α angle is 5° or less; and a step of applying a magnetic domain control treatment to the region where the absolute value of the α angle is 5° or less.

### (Step of measuring distribution of α angle)

First, the distribution of α angles on the surface of the original sheet of the grain-oriented electrical steel sheet 1 is measured. The α angle is measured by a side surface reflection Laue method described later.

The original sheet 2 is the grain-oriented electrical steel sheet 1 before the magnetic domain control treatment is applied.

### (Step of specifying region where absolute value of α angle is 5° or less)

Next, a region where the absolute value of the α angle is 5° or less on the surface of the original sheet is specified based on the distribution of the α angle. Hereinafter, a region where the absolute value of the α angle is 5° or less is referred to as a magnetic domain control treatment region 21.

### (Step of forming magnetic domain control treatment line)

FIG. 4 is a plan view of an example of the original sheet 2. FIG. 4 illustrates a magnetic domain control treatment region 21 and a non-magnetic domain control treatment region 22 of the original sheet 2. The magnetic domain control treatment is applied to the broken line illustrated in FIG. 4. The magnetic domain control treatment line can be formed using a known magnetic domain control treatment means. When the magnetic domain control treatment line 11 is a thermal strain, the magnetic domain control treatment may be executed by irradiation of the laser beam LB by the laser irradiation device 500, or other means such as ion implantation or electron beam irradiation may be adopted. When the magnetic domain control treatment line 11 is a groove, the magnetic domain control treatment may be executed using a tool for machining.

The control unit 513 of the laser irradiation device 500 performs control to turn on the power of the laser beam LB with respect to the magnetic domain control treatment region 21, and preferably, to turn off the power of the laser beam LB with respect to the non-magnetic domain control treatment region 22 (that is, a region other than the magnetic domain control treatment region 21). As a result, the magnetic domain control treatment line 11 is introduced into the magnetic domain control treatment region 21 of the original sheet 2. Further, in the non-magnetic domain control treatment region 22 of the original sheet 2, introduction of the magnetic domain control treatment line 11 is suppressed to a minimum.

### (Operation and Effects)

According to the above-described manufacturing method, it is possible to manufacture a steel sheet that achieves both iron loss reduction and noise reduction.

Although embodiments of the present invention have been described above, the present invention is not limited thereto, and can be appropriately modified without departing from the technical idea of the invention. Hereinafter, a more preferable example of the grain-oriented electrical steel sheet 1 according to the present embodiment and the method for manufacturing the same will be described. Unless otherwise specified, the preferred aspect described below is applicable to both the grain-oriented electrical steel sheet 1 and the method for manufacturing the same. As described later, the grain-oriented electrical steel sheet according to the present embodiment may have a forsterite film and/or an insulating coating on the surface of the base steel sheet.

Each will be described below. However, when the grain-oriented electrical steel sheet includes a base steel sheet and a forsterite film and/or an insulating coating, the following regulations regarding the chemical composition, the magnetic domain control treatment line, the magnetic domain control region, and the non-magnetic domain control treatment line are regulations regarding the base steel sheet. However, the provision regarding the sheet thickness is a provision regarding the entire grain-oriented electrical steel sheet including the base steel sheet, and the forsterite film and/or the insulating coating.

### (Chemical composition and sheet thickness)

The chemical compositions of the grain-oriented electrical steel sheet 1 and the original sheet 2 are not limited as long as they are equivalent to those of the known grain-oriented electrical steel sheet 1. For example, the chemical composition of the grain-oriented electrical steel sheet 1 and the original sheet 2 may be Si: 2.500 to 7.000%, Mn: 0.00 to 1.000%, C: 0 to 0.085%, acid-soluble Al: 0 to 0.065%, N: 0 to 0.012%, Cr: 0 to 0.300%, Cu: 0 to 0.400%, P: 0 to 0.500%, Sn: 0 to 0.300%, Sb: 0 to 0.300%, Ni: 0 to 1.000%, S: 0 to 0.015%, Se: 0 to 0.015%, Bi: 0 to 0.020%, Nb: 0 to 0.030%, V: 0 to 0.030%, Mo: 0 to 0.030%, Ta: 0 to 0.030%, W: 0 to 0.030%, B: 0 to 0.080%, and Ti: 0 to 0.015% in mass%. The balance of the chemical composition includes Fe and impurities.

The sheet thicknesses of the grain-oriented electrical steel sheet 1 and the original sheet 2 are not limited, but are preferably 0.15 to 0.30 mm, for example. When the thickness is 0.30 mm or less, classical eddy-current loss can be suppressed, and iron loss can be further improved. On the other hand, when the sheet thickness is 0.15 mm or more, rolling efficiency can be improved to improve productivity.

### (Surface treatment)

The grain-oriented electrical steel sheet 1 and the original sheet 2 may have a forsterite film. The grain-oriented electrical steel sheet 1 and the original sheet 2 may have an insulating coating. The forsterite film and the insulating coating may be formed on one surface or both surfaces of the grain-oriented electrical steel sheet 1.

The forsterite film is, for example, an inorganic coating film containing magnesium silicate as a main component. The forsterite film is formed, for example, by a reaction between an annealing separator containing magnesia (MgO) applied to the surface of the base steel sheet and a component of the surface of the base steel sheet in final annealing. The forsterite film has, for example, a composition (more specifically, a composition containing Mg₂SiO₄ as a main component) derived from the components of the annealing separator and the base steel sheet. On the other hand, when an annealing separator mainly containing Al₂O₃ is used in final annealing, a forsterite film may not be formed.

The insulating coating has a function of applying electrical insulation properties and tension to the grain-oriented electrical steel sheet 1. The tension is applied to the grain-oriented electrical steel sheet 1 to facilitate domain wall movement in the grain-oriented electrical steel sheet 1, and thus, the iron loss of the grain-oriented electrical steel sheet 1 can be reduced. In addition, according to the insulating coating, various characteristics such as corrosion resistance, heat resistance, and slippage can be provided to the grain-oriented electrical steel sheet 1. The insulating coating may be, for example, a known coating formed by applying a coating solution containing phosphate and colloidal silica as main components to the surface of the forsterite film and baking the coating solution.

The insulating coating is preferably formed after the final annealing and after the magnetic domain control treatment. On the other hand, the insulating coating may be formed after the final annealing step and before the magnetic domain control treatment. When the insulating coating is formed before the magnetic domain control treatment, the insulating coating may be peeled off in the magnetic domain control treatment line 11. Therefore, it is preferable to form the insulating coating again on the magnetic domain control treatment line 11 after the magnetic domain control treatment.

### (Angle formed by magnetic domain control treatment line 11 and transverse direction TD)

The angle formed by the magnetic domain control treatment line 11 and the transverse direction TD is not particularly limited. The magnetic domain control treatment line 11 and the transverse direction TD may be substantially parallel. That is, the angle formed by the magnetic domain control treatment line 11 and the transverse direction TD may be substantially 0°. On the other hand, as illustrated in FIG. 1, the angle formed by the magnetic domain control treatment line 11 and the transverse direction TD may be more than 0°. For example, the angle formed by the magnetic domain control treatment line 11 and the transverse direction TD may be an arbitrary value within the range of 0° to 45°. The angle formed by the magnetic domain control treatment line 11 and the transverse direction TD may be 1° or more, 3° or more, or 5° or more. The angle formed by the magnetic domain control treatment line 11 and the transverse direction TD may be 40° or less, 35° or less, or 30° or less.

As illustrated in FIG. 1, the angles formed by all the magnetic domain control treatment lines 11 and the transverse direction TD may be the same. That is, all the magnetic domain control treatment lines 11 may extend in parallel to each other. On the other hand, the angle formed by the magnetic domain control treatment line 11 and the transverse direction TD may vary. That is, some or all of a plurality of the magnetic domain control treatment lines 11 may extend non-parallel to each other. The average value of the angles formed by the magnetic domain control treatment line 11 and the transverse direction TD may be 1° or more, 3° or more, or 5° or more. The average value of the angles formed by the magnetic domain control treatment line 11 and the transverse direction TD may be 40° or less, 35° or less, or 30° or less. The average value of the angles may be calculated by measuring an angle formed with the transverse direction TD at a plurality of positions with respect to one magnetic domain control treatment line, or by measuring an angle formed with the transverse direction TD by a plurality of magnetic domain control treatment lines at one point or a plurality of positions.

### (Interval of magnetic domain control treatment line 11 along rolling direction RD)

The interval P along the rolling direction RD between the magnetic domain control treatment lines 11 adjacent along the rolling direction RD is not particularly limited. The effect of improving the iron loss is enhanced as the interval P is smaller. On the other hand, the larger the interval P, the more the noise characteristics are improved. The interval can be appropriately selected according to the characteristics required for the grain-oriented electrical steel sheet 1. For example, the interval P along the rolling direction RD between the magnetic domain control treatment lines 11 adjacent to each other along the rolling direction RD may be 1.0 mm or more, 2.0 mm or more, 3.0 mm or more, or 5.0 mm or more. The interval P along the rolling direction RD between the magnetic domain control treatment lines 11 adjacent along the rolling direction RD may be 10.0 mm or less, 9.0 mm or less, 8.0 mm or less, or 7.0 mm or less.

In the grain-oriented electrical steel sheet 1 exemplified in FIG. 1, the magnetic domain control treatment lines 11 are provided at regular intervals. On the other hand, the interval P along the rolling direction RD between the magnetic domain control treatment lines 11 adjacent along the rolling direction RD may vary. For example, the average value of the interval P along the rolling direction RD between the magnetic domain control treatment lines 11 adjacent to each other along the rolling direction RD may be 1.0 mm or more, 2.0 mm or more, 3.0 mm or more, or 5.0 mm or more. The average value of the intervals P along the rolling direction RD between the magnetic domain control treatment lines 11 adjacent along the rolling direction RD may be 10.0 mm or less, 9.0 mm or less, 8.0 mm or less, or 7.0 mm or less.

### (Magnitude of tensile stress introduced in thermal strain)

The magnetic domain control treatment line 11 may be due to a thermal strain. In the thermal strain, tensile stress is introduced. As the tensile stress is larger, the effect of improving the iron loss is enhanced. On the other hand, as the tensile stress is smaller, the noise characteristics are improved. Tensile stress according to characteristics required for the grain-oriented electrical steel sheet 1 can be appropriately selected.

The magnitude of the tensile stress is not particularly limited, but for example, in at least a part of the magnetic domain control treatment line 11, the tensile stress in an arbitrary direction is preferably 40 MPa or more, 60 MPa or more, or 80 MPa or more. When the tensile stress in at least one direction is 40 MPa or more, it is considered that the requirement that "the tensile stress in an arbitrary direction is 40 MPa or more" is satisfied. For example, in at least a part of the magnetic domain control treatment line 11, the tensile stress in an arbitrary direction is preferably 300 MPa or less, 200 MPa or less, 180 MPa or less, or 150 MPa or less. The tensile stress in an arbitrary direction in the magnetic domain control treatment line 11 may be uniform or may vary.

### (Depth and width of groove)

The magnetic domain control treatment line 11 may be a groove. As the depth and width of the groove are larger, the effect of improving the iron loss is enhanced. On the other hand, the noise characteristics are improved as the depth and width of the groove are smaller. The shape of the groove can be appropriately selected according to the characteristics required for the grain-oriented electrical steel sheet 1.

The depth of the groove is not particularly limited, but is preferably, for example, 5 µm to 50 µm. The depth of the groove may be 6 µm or more, 7 µm or more, or 10 µm or more. The depth of the groove may be 48 µm or less, 45 µm or less, or 40 µm or less.

The width of the groove (width at the opening part) is not particularly limited, but is preferably, for example, 10 µm to 300 µm. The width of the groove may be defined as 20 µm or more, 30 µm or more, or 50 µm or more. The width of the groove may be defined as 280 µm or less, 250 µm or less, or 200 µm or less. The depth and width of the groove may be uniform or may vary. In the case of variation, the average of the depths and widths of a plurality of the grooves is preferably in the above range.

### (Number of magnetic domain control points)

As the number of magnetic domain control points increases, the number of magnetic domain control treatment lines increases, and the region subjected to the magnetic domain control treatment increases. Therefore, from the viewpoint of iron loss reduction, it is preferable that the number of magnetic domain control points is large. For example, the number of magnetic domain control points in the grain-oriented electrical steel sheet 1 is preferably 10 points or more, 50 points or more, or 100 points or more per 10,000 mm².

### (Measurement method)

Hereinafter, a method for measuring various parameters of the grain-oriented electrical steel sheet 1 according to the present embodiment will be described. Measurement of any parameter is performed on a sample collected from the grain-oriented electrical steel sheet 1. For example, a rectangular sample having both sides of 100 mm (or 100 mm or more) in length can be cut out from the grain-oriented electrical steel sheet 1 and subjected to measurement. When the grain-oriented electrical steel sheet 1 is a coil, a sample may be collected from an arbitrary position of the coil. When the grain-oriented electrical steel sheet 1 is a component incorporated in an electrical product such as a transformer or a motor, a sample may be collected from any place of the component. When the size of the component is small, the length of one side of the sample may be less than 100 mm. In this case, the total value of the sample areas is set to 10,000 mm² or more. At that time, it is desirable to collect a sample by a method such as wire cutting in order to minimize the influence of mechanical strain or the like on the sample.

### (Method of identifying magnetic domain control treatment line 11)

When the magnetic domain control treatment line 11 is a groove, the magnetic domain control treatment line 11 can be visually identified. When the grain-oriented electrical steel sheet 1 has an insulating coating, the magnetic domain control treatment line 11 becomes visible by removing the insulating coating using a known peeling agent.

When the magnetic domain control treatment line 11 is a thermal strain, the magnetic domain control treatment line 11 may not be visually identified. In this case, for example, the magnetic domain image is photographed using an image acquisition device. If necessary, a magnetic domain image is photographed while a DC magnetic field is applied along the rolling surface normal direction ND of the grain-oriented electrical steel sheet 1. The position of the thermal strain can be identified by observing the magnetic domain image.

### (Method for specifying rolling direction RD and transverse direction TD)

The rolling direction RD and the transverse direction TD of the grain-oriented electrical steel sheet 1 are specified by the following means.
(1) When the sample is cut out from the coil-shaped grain-oriented electrical steel sheet 1, the width direction of the coil is regarded as the transverse direction TD. A direction perpendicular to the transverse direction TD and the rolling surface normal direction ND is regarded as the rolling direction RD.
(2) When the sample is cut out from a part or the like of an electrical product, the rolling direction RD and the transverse direction TD are specified from rolling defects on the surface of the grain-oriented electrical steel sheet 1. The extending direction of the rolling defect is regarded as a rolling direction RD. A direction perpendicular to the rolling direction RD and the rolling surface normal direction ND is regarded as a transverse direction TD.
(3) When it is difficult to specify the rolling direction RD and the transverse direction TD from a rolling defect on the surface of the grain-oriented electrical steel sheet 1, the rolling direction RD and the transverse direction TD are specified from the crystal orientation of the grain-oriented electrical steel sheet 1. Specifically, the crystal orientation of the grain-oriented electrical steel sheet 1 to be evaluated is measured at a plurality of points. Then, the direction in which the deviation angle from the magnetization easy axis <001> at which the angle formed by the crystal orientation at the measurement point with the rolling surface normal direction ND (sheet thickness direction) is the closest to the right angle is minimized is regarded as the rolling direction RD, and the direction perpendicular to the rolling direction RD and the rolling surface normal direction ND is regarded as the transverse direction TD.

### (Method of measuring α angle and γ angle)

The α and γ angles are measured by the side surface reflection Laue method. The side surface reflection Laue method is widely known as a method for measuring a crystal orientation. However, the α angle and the γ angle are values obtained by rounding off the measured numerical value to the first decimal place. That is, the significant digits of the α angle and the γ angle are set to the first decimal place.

### (Method of measuring distribution of α angle)

The method for measuring the distribution of α angles on the surface of the original sheet of the grain-oriented electrical steel sheet 1 is as follows. Measurement points are set in a grid shape on the surface of the original sheet of the grain-oriented electrical steel sheet 1. At each measurement point, the α angle is measured.

Specifically, measurement points are set in a grid pattern at an interval of 2 mm along the rolling direction RD and the transverse direction TD with respect to the surface of the original sheet of the grain-oriented electrical steel sheet 1. The α angle is measured at each measurement point, and the distribution of the α angle on the surface of the original sheet of the grain-oriented electrical steel sheet 1 is measured.

### (Calculation method of |α_{All}|)

An outline of a method of calculating |α_{All}| is as follows. As illustrated in FIG. 5, measurement points are set in a grid pattern on the surface of a sample collected from the grain-oriented electrical steel sheet 1. The absolute value of the α angle is measured at each measurement point, and the average value thereof is calculated. This average value is regarded as |α_{All}|.

Specifically, an imaginary line VL1 parallel to the transverse direction TD and an imaginary line VL2 parallel to the rolling direction RD are set for the surface of the sample (rectangular region surrounded by alternate long and short dash line in FIG. 5) having one side of 100 mm or more. In setting the imaginary line VL1 and the imaginary line VL2, the presence of the magnetic domain control treatment line 11 is not considered. The interval between the imaginary lines VL1 is set to 2 mm. The interval between the imaginary lines VL2 is set to 2 mm. The imaginary line VL1 and the imaginary line VL2 are arranged over the entire surface of the sample. The absolute value of the α angle at the intersection point VP1 of the imaginary line VL1 and the imaginary line VL2 is measured.

### (Calculation method of |α_{Dr}|)

A method of calculating |α_{Dr}| is as follows. First, on the surface of a sample (rectangular region surrounded by alternate long and short dash line in FIG. 1 or 2) having a side of 100 mm or more, a plurality of the imaginary lines VL3 are set at regular intervals in parallel along the rolling direction RD of the grain-oriented electrical steel sheet 1. VL3 may be the same as or different from imaginary line VL2 parallel to rolling direction RD at the time of calculating |α_{All}|. The interval between the imaginary lines VL3 is 2 mm. The imaginary line VL3 is arranged over the entire surface of the sample. Next, the magnetic domain control point VP2 (that is, the intersection point of the imaginary line VL3 and the magnetic domain control treatment line 11) is specified. Then, the absolute value of the α angle at each magnetic domain control point VP2 is measured, and the average value thereof is calculated. This average value is regarded as |α_{Dr}|. The method of specifying the rolling direction RD and the magnetic domain control treatment line 11 and the method of measuring the α angle are as described above.

### (Method of measuring σα_{All})

σα_{All} is obtained by calculating the standard deviation of the absolute value of the α angle at each measurement point used to calculate |α_{All}|. The method for specifying the absolute value of the α angle at each measurement point is as described above.

### (Method for measuring σα_{Dr})

σα_{Dr} is obtained by calculating the standard deviation of the absolute value of the α angle at each magnetic domain control point VP2. The method for specifying the magnetic domain control point VP2 is as described above.

### (Calculation method of |γ_{All}|)

An outline of a method of calculating |γ_{All}| is as follows. As illustrated in FIG. 5, measurement points are set in a grid pattern at intervals of 2 mm along the rolling direction RD and the transverse direction TD on the surface of the sample collected from the grain-oriented electrical steel sheet 1. The absolute value of the γ angle is measured at each measurement point, and the average value thereof is calculated. This average value is regarded as |γ_{All}|.

### (Method for measuring chemical components of original sheet 2 and grain-oriented electrical steel sheet 1)

The chemical compositions of the grain-oriented electrical steel sheet 1 and the original sheet 2 may be measured by a general analysis method of steel. For example, the chemical component may be measured using inductively coupled plasma-atomic emission spectrometry (ICP-AES). Specifically, the chemical composition of the grain-oriented electrical steel sheet 1 and the original sheet 2 can be measured by acquiring a test piece from the center portion in the thickness direction of the sample, and measuring the test piece under a condition based on a calibration curve prepared in advance using ICPS-8100 manufactured by Shimadzu Corporation or the like (measuring device). The amounts of C and S, which are difficult to measure by ICP-AES, may be measured using a combustion-infrared light absorption method. The amount of N may be measured using an inert gas fusion-thermal conductivity method.

When the forsterite film and/or the insulating coating are/is formed on the grain-oriented electrical steel sheet 1, the chemical component of the grain-oriented electrical steel sheet 1 (that is, the chemical composition of the base steel sheet) may be analyzed after removing the forsterite film and/or the insulating coating from the grain-oriented electrical steel sheet 1. The insulating coating can be removed, for example, by immersing the sample in a sodium hydroxide solution and then immersing the sample in dilute sulfuric acid and nitric acid. Conditions such as the temperature and concentration of sodium hydroxide, dilute sulfuric acid, and nitric acid solution, and the time for immersion are appropriately adjusted so that the base metal of the sample is not excessively dissolved. An example of the conditions of the removal operation of the insulating coating is as follows. First, the sample is immersed in a sodium hydroxide solution having a concentration of 20% at 80°C for 15 minutes. Thereafter, the sample is dried. Then, the sample is immersed in diluted sulfuric acid having a concentration of 10% at 80°C for 4 minutes. Thereafter, the sludge adhering to the surface of the sample is removed with a waste cloth or the like. Further, the sample is immersed in nitric acid having a concentration of 10% at room temperature while being stirred for about 10 seconds.

The forsterite film can be removed, for example, by immersing the sample in sulfuric acid followed by immersion in nitric acid. Conditions such as the temperature and concentration of sulfuric acid and nitric acid and the time for immersion are appropriately adjusted so that the base metal of the sample is not excessively dissolved. An example of conditions of the removal operation of the forsterite film is as follows. First, the sample is immersed in sulfuric acid having a concentration of 10% at 80°C for 3 minutes. Thereafter, the surface of the sample is washed with water using a waste cloth or the like to remove the sludge adhering to the surface. Thereafter, the sample is dried. Further, the sample is immersed in nitric acid having a concentration of 10% at room temperature while being stirred for about 5 seconds.

### (Method of measuring angle formed by magnetic domain control treatment line 11 and transverse direction TD)

The angle formed by the magnetic domain control treatment line 11 and the transverse direction TD can be measured using a known angle measuring means after the magnetic domain control treatment line 11 and the transverse direction TD are specified by the above-described procedure.

### (Method for measuring interval of magnetic domain control treatment line 11 along rolling direction RD)

The interval of the magnetic domain control treatment line 11 along the rolling direction RD can be measured using a known length measuring means after the magnetic domain control treatment line 11 and the rolling direction RD are specified by the above-described procedure.

### (Method for measuring magnitude of tensile stress introduced in thermal strain)

The magnitude of the tensile stress introduced in the thermal strain is measured by the EBSD Wilkinson method and Cross Court manufactured by BLG Vantage. The EBSD Wilkinson method is described in detail in A.J.Wilkinson, et al. "High-resolution elastic strain measurement from electron backscatter diffraction patterns: New levels of sensitivity" Ultramicroscopy Vol 106, No. 4-5, March 2006, P. 307-313.

When the magnitude of the tensile stress introduced in the thermal strain is measured by the EBSD Wilkinson method and the Cross Court manufactured by BLG Vantage, first, the magnetic domain control treatment line 11 is specified by the above-described procedure. Next, the grain-oriented electrical steel sheet 1 is cut through the magnetic domain control treatment line 11 and perpendicularly to the magnetic domain control treatment line 11. This cut cross section is used as a measurement surface. The cross section of the magnetic domain control treatment line 11 included in the measurement surface is analyzed by the EBSD Wilkinson method and Cross Court manufactured by BLG Vantage, and a tensile stress component in an arbitrary direction is extracted and the magnitude thereof is measured. For example, it is possible to extract a tensile stress component in a rolling surface normal direction ND, a direction parallel to the magnetic domain control treatment line 11, and a direction perpendicular to the rolling surface normal direction ND and the magnetic domain control treatment line 11.

The number of measurement points is, for example, 10. When the tensile stress in an arbitrary direction is 40 MPa or more (that is, when the tensile stress in at least one direction is 40 MPa or more,) in at least one location of the grain-oriented electrical steel sheet 1, the absolute maximum value of the tensile stress in an arbitrary direction in the magnetic domain control treatment line of the grain-oriented electrical steel sheet 1 is determined to be 40 MPa or more. When a measurement point at which the tensile stress in any direction is 40 MPa or more is found, the measurement of the tensile stress may be stopped.

### (Method of measuring depth and width of groove)

The depth and width of the groove can be measured by specifying the surface shape of the sample using a known three-dimensional measuring machine. When the grain-oriented electrical steel sheet 1 has a tension insulation coating, the insulating coating is removed by the above-described procedure, and then the three-dimensional measurement of the sample surface is performed.

### Examples

The effect of one aspect of the present invention is described more specifically with reference to examples. However, the conditions in the examples are merely one condition example adopted to confirm the operability and effects of the present invention. The present invention is not limited to this one condition example. The present invention can adopt various conditions as long as the object of the present invention is achieved without departing from the gist of the present invention.

A grain-oriented electrical steel sheet of the same lot having a sheet thickness of 0.20 mm was used as the original sheet. The original sheet was subjected to a magnetic domain control treatment under various conditions shown in Table 1. The noise and iron loss of the grain-oriented electrical steel sheets subjected to the magnetic domain control treatment obtained as a result are evaluated and described in Table 2. In Table 1, values outside the range of the grain-oriented electrical steel sheet according to the present embodiment are underlined. In Table 2, values that do not satisfy the following pass/fail criteria are underlined.

The methods for evaluating noise and iron loss were as follows. First, 205 grain-oriented electrical steel sheets having a sheet thickness of 0.20 mm were laminated to form a three-phase transformer core. The widths of the foot and the yoke of the three-phase transformer core were both 150 mm. The height and width of the outer shape of the three-phase transformer core were both 750 mm. Noise and iron loss of these three-phase transformer cores were measured. The measurement conditions were a frequency of 60 Hz and an excitation magnetic flux density of 1.8 T.

In measuring the noise, microphones were arranged at equal intervals at eight points around the transformer in which the three-phase transformer core was incorporated. The distance between the transformer and the microphone was 30 cm. The values obtained by correcting the A characteristics to the noise measurement results by the microphones and averaging the results are described in Table 2 as the noise evaluation results (unit: dBA) of the grain-oriented electrical steel sheets. An example in which the evaluation result of noise was 51.00 dBA or less was determined to be an example in which noise reduction was achieved. The noise evaluation result determined to be unacceptable was underlined.

The iron loss was obtained by measuring voltages and currents on the primary side and the secondary side with a power analyzer when excitation was performed at a frequency of 60 Hz and an excitation magnetic flux density of 1.8 T as described above. The obtained iron loss is described in Table 2 as an iron loss evaluation result (unit: W/kg) of the grain-oriented electrical steel sheet. An example in which the evaluation result of the iron loss was 1.270 W/kg or less was determined to be an example in which iron loss reduction was achieved. The noise evaluation result determined to be unacceptable was underlined.

Further, |α_{All}|, |α_{Dr}|, |γ_{All}|, σα_{All}, and σα_{Dr} in the grain-oriented electrical steel sheets subjected to the magnetic domain control treatment were measured and described in Table 2. The measurement method was in principle according to the procedure described above. A rectangular sample having both sides of 100 mm in length was cut out from a three-phase transformer core for measuring noise and iron loss, and subjected to measurement.

**[Table 1]**

| Example No. | \|α_{All}\|-\|α_{Dr}\| | \|γ_{All}\|-\|α_{Dr}\| | σα_{All} | σα_{Dr} | Type of magnetic domain control treatment line | Remarks |
|---|---|---|---|---|---|---|
| 1 | 0.1 | -0.6 | 1.5 | 1.6 | Thermal strain | Treatment line in region where the α angle is small |
| 2 | 0.1 | -1.2 | 1.5 | 1.6 | Groove | Treatment line in region where the α angle is small |
| 3 | 0.1 | -0.8 | 1.5 | 1.6 | Mixed | Treatment line in region where the α angle is small |
| 4 | 0.2 | -0.8 | 1.2 | 1.3 | Thermal strain | Treatment line in region where the α angle is small |
| 5 | 0.4 | -0.9 | 1.2 | 1.2 | Thermal strain | Treatment line in region where the α angle is small |
| 6 | 1.1 | 0.4 | 1.2 | 1.2 | Thermal strain | Treatment line in region where the α angle is small |
| 7 | 2.7 | 1.7 | 1.5 | 1.5 | Thermal strain | Treatment line in region where the α angle is small |
| 8 | 1.5 | 0.8 | 0.8 | 1 | Thermal strain | Treatment line in region where the α angle is small |
| 9 | 1.7 | 1.2 | 1.4 | 0.8 | Thermal strain | Treatment line in region where the α angle is small |
| 10 | 0 | 0 | 1.5 | 1.5 | Thermal strain | straight line treatment line over the entire width |
| 11 | 0 | 0 | 1.4 | 1.4 | Thermal strain | Random broken-line treatment line |
| 12 | 0 | 0 | 1.3 | 1.3 | Thermal strain | Regular dashed-line treatment line |
| 13 | -0.5 | -0.8 | 1.2 | 1.6 | Thermal strain | Treatment line in region where the α angle is large |
| 14 | -0.5 | -0.8 | 1.2 | 1.4 | Thermal strain | Treatment line in region where the α angle is large |

**[Table 2]**

| Example No. | Evaluation results of noise | Evaluation results of iron loss |
|---|---|---|
| 1 | 51.0 | 1.240 |
| 2 | 50.3 | 1.266 |
| 3 | 50.7 | 1.250 |
| 4 | 48.5 | 1.249 |
| 5 | 46.1 | 1.254 |
| 6 | 44.2 | 1.263 |
| 7 | 43.9 | 1.267 |
| 8 | 44.0 | 1.247 |
| 9 | 41.9 | 1.245 |
| 10 | 56.7 | 1.239 |
| 11 | 55.8 | 1.270 |
| 12 | 55.6 | 1.273 |
| 13 | 49.3 | 1.293 |
| 14 | 42.6 | 1.294 |

In Example No. 10, all the magnetic domain control treatment lines were formed over the entire width of the grain-oriented electrical steel sheet. As a result, Example No. 10 did not satisfy |α_{All}|-|α_{Dr}| ≥ 0.1°. In Example No. 10, the iron loss was within the acceptable range, but the noise characteristics were unacceptable.

In Example No. 11, the magnetic domain control treatment line was formed in a broken line shape. That is, in Example No. 11, similarly to Example No. 1 to 9, a region where the magnetic domain control treatment is not performed is provided. However, in Example No. 11, the sizes of the gaps between the magnetic domain control treatment lines included in the broken line were randomly varied. Portions where the magnetic domain control treatment was not performed were randomly provided. As a result, Example No. 11 did not satisfy |α_{All}|-|α_{Dr}| ≥ 0.1°. In Example No. 11, the iron loss was within the acceptable range, but was the same value as 1.270 which is the acceptance determination value. In addition, in Example No. 11, the noise characteristics were unacceptable.

In Example No. 12, the magnetic domain control treatment lines were formed in an ordered broken line shape. That is, in Example No. 12, similarly to Example No. 1 to 9, a region where the magnetic domain control treatment is not performed is provided. However, in Example No. 12, the size of the gap between the magnetic domain control treatment lines included in the broken line is set to a constant value. Portions where the magnetic domain control treatment was not performed were regularly provided. As a result, Example No. 12 did not satisfy |α_{All}|-|α_{Dr}| ≥ 0.1°. In Example No. 12, both the iron loss and the noise characteristic were unacceptable.

Also in Example No. 13 and Example No. 14, similarly to Example No. 11, the magnetic domain control treatment line was formed in a broken line shape. That is, in Example No. 13 and Example No. 14, similarly to Examples No. 1 to 9, a region where the magnetic domain control treatment is not performed is provided. However, in Example No. 13 and Example No. 14, the magnetic domain control treatment is applied to a region where the α angle is larger than a predetermined value, limited on the basis of the distribution of the α angle. These examples also did not satisfy |α_{All}|-|α_{Dr}| ≥ 0.1°. In Example No. 13 and Example No. 14, the iron loss was unacceptable.

On the other hand, in Examples No. 1 to 9, the magnetic domain control treatment is applied to a region where the α angle is a predetermined value or less, limited on the basis of the distribution of the α angle. Examples No. 1 to 9 satisfied |α_{All}|-lα_{Dr}| ≥ 0.1°, and both the noise characteristics and the iron loss fell within the acceptable range. By Examples Nos. 1 to 9, both iron loss reduction and noise reduction were achieved.

According to Examples No. 1 to 9, it was confirmed that the larger |α_{All}|-|α_{Dr}|, the better the noise characteristics. In Examples No. 6 to 9, |γ_{All}|-|α_{Dr}| ≥ 0.1° was satisfied. In these examples, the noise characteristics were further excellent. In Example No. 9, |γ_{All}|-|α_{Dr}| ≥ 0.1° was satisfied, and σα_{Dr} < σα_{All} was satisfied. In this example, the noise characteristics were further excellent.

### INDUSTRIAL APPLICABILITY

Since the hot-rolled steel sheet of the present disclosure can achieve both iron loss reduction and noise reduction, the hot-rolled steel sheet has high industrial applicability.

### REFERENCE SIGNS LIST

1 Grain-oriented electrical steel sheet
11 Magnetic domain control treatment line
12A Region where the α angle is small
12B Region where the α angle is large
RD Rolling direction
TD Transverse direction
ND Rolled surface normal direction
VL1 Imaginary line parallel to TD for |α_{All}| calculation
VL2 Imaginary line parallel to RD for |α_{All}| calculation
VL3 Imaginary line parallel to TD for |α_{Dr}| calculation
VP1 Intersection point of imaginary line VL1 and imaginary line VL2
VP2 Magnetic domain control point
2 Original sheet
21 Magnetic domain control treatment region
22 Non-magnetic domain control treatment region
30 Image acquisition device
31 Light Source Unit
500 Laser irradiation device
501 Polygon mirror
503 light source device
505 Collimator
507 Condensing lens
509 Motor
511 Sensor
513 Control unit
515 Sheet passing device

## Claims

1. A grain-oriented electrical steel sheet having a magnetic domain control treatment line on a surface thereof, wherein
|α_{All}|-|α_{Dr}| ≥ 0.1° is satisfied,
|α_{All}| is an average value of absolute values of α angles over an entire surface of the grain-oriented electrical steel sheet, and
|α_{Dr}| is an average value of absolute values of α angles at magnetic domain control points that are intersection points of a plurality of the imaginary lines set at intervals of 2 mm in parallel along a rolling direction of the grain-oriented electrical steel sheet and the magnetic domain control treatment line.

2. The grain-oriented electrical steel sheet according to claim 1, wherein |α_{All}|-lα_{Dr}| ≥ 0.2° is satisfied.

3. The grain-oriented electrical steel sheet according to claim 1, wherein |α_{All}|-lα_{Dr}| ≥ 0.5° is satisfied.

4. The grain-oriented electrical steel sheet according to claim 1, wherein |α_{All}|-lα_{Dr}| ≥ 1.0° is satisfied.

5. The grain-oriented electrical steel sheet according to any one of claims 1 to 4, wherein
|γ_{All}|-|α_{Dr}| ≥ 0.1° is satisfied,
|γ_{All}| is an average value of absolute values of y angles over the entire surface of the grain-oriented electrical steel sheet.

6. The grain-oriented electrical steel sheet according to any one of claims 1 to 4, wherein
σα_{Dr} < σα_{All} is satisfied,
σα_{All} is a standard deviation of the absolute value of the α angle over the entire surface of the grain-oriented electrical steel sheet, and
σα_{Dr} is the standard deviation of the absolute value of the α angle at the magnetic domain control point.

7. The grain-oriented electrical steel sheet according to any one of claims 1 to 4, wherein the magnetic domain control treatment line is a groove.

8. A method for manufacturing a grain-oriented electrical steel sheet comprising:
a step of measuring a distribution of α angles on a surface of an original sheet of a grain-oriented electrical steel sheet;
a step of specifying a region where an absolute value of the α angle is 5° or less; and
a step of forming a magnetic domain control treatment line in the region where the absolute value of the α angle is 5° or less.

9. The method for manufacturing a grain-oriented electrical steel sheet according to claim 8, wherein a magnetic domain control treatment is applied by irradiation with a laser or an electron beam.
